



US006136492A

# United States Patent [19]

Hardy, Jr. et al.

[11] Patent Number: 6,136,492

[45] Date of Patent: Oct. 24, 2000

[54] **TONER RESIN FOR LIQUID TONER COMPOSITIONS**

[75] Inventors: **Gordon Edward Hardy, Jr.**, Hudson; **Gary Lee Burroway**, Doylestown, both of Ohio

[73] Assignee: **The Goodyear Tire & Rubber Company**, Akron, Ohio

[21] Appl. No.: 09/243,239

[22] Filed: Feb. 3, 1999

## Related U.S. Application Data

[60] Provisional application No. 60/085,277, May 13, 1998.

[51] Int. Cl. 7 G03G 9/087; G03G 9/135

[52] U.S. Cl. 430/115; 430/109; 430/114

[58] Field of Search 526/329.1; 430/114 430/109, 115

## [56] References Cited

### U.S. PATENT DOCUMENTS

|           |         |                     |           |
|-----------|---------|---------------------|-----------|
| 4,298,672 | 11/1981 | Lu                  | 430/108   |
| 4,338,390 | 7/1982  | Lu                  | 430/106   |
| 4,450,260 | 5/1984  | Von Bodungen et al. | 526/213   |
| 4,469,770 | 9/1984  | Nelson              | 430/110   |
| 4,544,726 | 10/1985 | Alford et al.       | 526/309   |
| 5,247,034 | 9/1993  | Mate et al.         | 526/215   |
| 5,852,151 | 12/1998 | Burroway et al.     | 526/329.1 |

Primary Examiner—John Goodrow

Attorney, Agent, or Firm—Alvin T Rockhill

## [57] ABSTRACT

This invention is based upon the discovery that the characteristics of toner resins made by emulsion polymerization can be improved by utilizing diacid cycloaliphatic emulsifiers in the synthesis thereof. Toner resins which are made utilizing such diacid cycloaliphatic emulsifiers do not exhibit significant electrical charge effects from the residual level of soap in the resin compared to resins made using standard soaps; such as, rosin acid soaps and fatty acid soaps. They also generally contain a lower level of ash since salts do not need to be used in their coagulation. As a result of the low level of ash, the toner resin made from the diacid soap exhibits excellent resistance to moisture sensitivity and adsorption. This feature gives the toners made from these resins better electrical charge stability compared to resins made from conventional soaps since adsorbed moisture is known to neutralize electrical charges. Solid and liquid toners made from these resins also exhibit greatly improved adhesion to paper. This invention more specifically discloses a process for preparing a polymer which is particularly useful as a toner resin, which comprises (1) emulsion copolymerizing a vinyl aromatic monomer and a second monomer selected from the group consisting of conjugated diene monomers and an acrylate monomer selected from the group consisting of alkyl acrylate monomers and methacrylate monomers in the presence of a diacid cycloaliphatic emulsifier to produce the polymer and (2) recovering the polymer from the aqueous emulsion.

42 Claims, No Drawings

## TONER RESIN FOR LIQUID TONER COMPOSITIONS

This application claims the benefit of U.S. Provisional Patent Application Serial No. 60/085,277, filed on May 13, 1998.

### BACKGROUND OF THE INVENTION

The development of electrostatic latent images with toner particles is well known. Over the years, the level of sophistication achieved in the field of electrostatic latent image development systems has been remarkable. For example, slow and laborious manual systems commercialized in the late 1950s have evolved into elegant high speed development systems creating as many as three copies per second. Consequently, the performance standards for toners during the evolution of electrostatography have become increasingly stringent. In the early manual development systems, toner and carrier particles were merely moved over an imaging surface bearing an electrostatic latent image by hand, tilting a tray containing the imaging surface, toner and carrier particles. However, in recent years, toner particles are automatically recycled many thousands of times over imaging surfaces moving at extremely high velocities. Thus, durable toner materials are required to withstand the physical punishment of vigorous, prolonged and continuous use. Moreover, toner particles deposited in image configuration must now be fused in extremely short periods of time.

Due to the size limitations of electrostatic copying and printing machines, the fusing path must be relatively short. When one attempts to increase the heat energy applied to deposited toner images for fusing purposes within the constraints of a limited fusing path to achieve adequate fixing at higher rates, one approaches the charring or kindling temperature of the substrate bearing the toner image. Attempts to shorten the fusing path by utilizing flash fusing techniques often result in the formation of noxious fumes due to decomposition of components in some toners. Further, the cost and availability of energy to operate an electrostatographic imaging system is of increasing concern to users. In addition, toner materials must possess the proper triboelectric charging properties for electrostatic latent image development and must not agglomerate during storage and transportation. Thus, there is a great need for an improved toner having stable electrical and physical properties which can endure the harsh environment of high speed electrostatographic copiers and printers and which can also be fused at lower temperatures utilizing less energy.

It is well known that electrostatic latent images can be developed with toner compositions which are comprised of a melt blend of toner resin and pigment particles. In such systems, negatively charged toner particles are generally selected for the development of positively charged electrostatic latent images. However, in recent years, the use of positively charged toner compositions containing charge enhancing additives for the purpose of imparting positive charge to toner resin particles has become more popular. These positively charged toner compositions are particularly useful for causing the development of negatively charged electrostatic latent images formed on layered organic photoreceptor imaging members. Examples of positively charged toner compositions useful for causing the development of negatively charged electrostatic latent images are disclosed in U.S. Pat. No. 4,298,672, U.S. Pat. No. 4,338,390 and U.S. Pat. No. 4,469,770.

Certain copolymers of styrene and butadiene have been developed which meet the demanding requirements of posi-

tively charged toner compositions. Such styrene-butadiene copolymers can be made by various techniques with emulsion polymerization being the most common. However, there are a number of traditional drawbacks associated with utilizing emulsion polymerization in preparing such toner resins which are utilized in preparing toners designed to build stable charge. For instance, undesirable residual contaminants are typically present in toner resins made by emulsion polymerization. In many cases, these residual contaminants have a very detrimental effect on the performance characteristics of the toner resin.

Rosin acids and fatty acids are commonly utilized as emulsifiers in preparing toner resins by emulsion polymerization. The presence of residual rosin acids and residual fatty acids in toner resins limits their ability to build stable electrical charges. The coagulants utilized in recovering the resin from the aqueous emulsion are also generally present as residual contaminants in such toner resins. The presence of ash from the coagulants also limits the ability of toners made utilizing such resins to build a stable charge. For these reasons, emulsion polymerization has typically been considered to be inferior to solution polymerization and suspension polymerization techniques for synthesizing such toner resins.

U.S. Pat. No. 5,247,034 discloses the utilization of amino acid soaps in the synthesis of toner resins and circumvents some of the problems associated with utilizing rosin acid soaps or fatty acid soaps. By virtue of the fact that such emulsions can be coagulated without the utilization of salts, the resins made by the process disclosed in U.S. Pat. No. 5,247,034 exhibit low levels of residual ash. This is advantageous in that the presence of ash reduces the level of charge which can be realized. As a result of the low level of ash, the toner resin made utilizing the amino acid soap exhibits excellent resistance to moisture sensitivity and adsorption. This feature gives toners made from these resins better electrical charge stability compared to resins made from other soaps since adsorbed moisture is known to neutralize electrical charges. However, toners made with resins synthesized utilizing the technique of U.S. Pat. No. 5,247,034 have low adhesion characteristics to paper.

### SUMMARY OF THE INVENTION

The key to this invention is the utilization of a diacid cycloaliphatic emulsifier in synthesizing the toner resin. This circumvents some of the problems associated with utilizing rosin acid soaps or fatty acid soaps. By virtue of the fact that such emulsions can be coagulated without the utilization of salts, the resins made by the process of this invention exhibit low levels of residual ash. This is advantageous in that the presence of ash reduces the level of charge which can be realized. As a result of the low level of ash, the toner resin made utilizing the diacid cycloaliphatic emulsifier exhibits excellent resistance to moisture sensitivity and adsorption. This feature gives toners made from these resins better electrical charge stability compared to resins made from standard soaps since adsorbed moisture is known to neutralize electrical charges.

Solid and liquid toners made with resins synthesized utilizing the technique of this invention also exhibit greatly improved adhesion to paper. This is highly desirable since it allows for printers and copiers to operate at a lower fusion temperature which results in energy savings. Better adhesion characteristics also normally allow for printers and copiers to be operated at greater speeds.

By utilizing the process of this invention, toner resins can be prepared which are of a very high quality. These toner

resins can be utilized in making toners which are capable of building very stable charges without compromising adhesion characteristics. Heretofore, it was only possible to make toner resins having such physical characteristics by solution polymerization or suspension polymerization routes.

This invention more specifically describes a process for preparing a polymer which is particularly useful as a toner resin, which comprises (1) emulsion copolymerizing a vinyl aromatic monomer and a second monomer selected from the group consisting of conjugated diene monomers and an acrylate monomer selected from the group consisting of alkyl acrylate monomers and alkyl methacrylate monomers in the presence of a diacid cycloaliphatic emulsifier to produce the polymer and (2) recovering the polymer from the aqueous emulsion. The polymer is normally recovered from the aqueous emulsion by coagulating the emulsion with an acid, such as sulfuric acid. The coagulation will normally be carried out in the absence of salts, such as sodium chloride or potassium chloride, to keep the level of ash low.

The present invention also discloses a toner resin which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers and (b) a residual amount of a diacid cycloaliphatic emulsifier. It is highly desirable for the toner resin not to contain residual levels of other emulsifiers, such as rosin acid soaps or fatty acid soaps.

The subject invention further discloses a solid toner composition which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers, (b) a residual amount of a diacid cycloaliphatic emulsifier and (c) a pigment. The toner can optionally further contain a charge control agent and/or a wax.

The present invention also reveals a liquid toner composition which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers, (b) a residual amount of a diacid cycloaliphatic emulsifier, (c) a pigment and (d) a carrier liquid.

#### DETAILED DESCRIPTION OF THE INVENTION

The toner resins made by utilizing the process of this invention are comprised of repeat units which are derived from a vinyl aromatic monomer and a second monomer selected from the group consisting of conjugated diene monomers and alkyl acrylate monomers. These polymers are, accordingly, made by copolymerizing the vinyl aromatic monomer with a conjugated diene monomer or an alkyl acrylate monomer. The conjugated diene monomers which can be used typically contain from 4 to about 10 carbon atoms. As a general rule, the conjugated diene monomer will contain from 4 to about 6 carbon atoms. Isoprene and 1,3-butadiene are highly preferred conjugated diene monomers for utilization in making toner resins by the process of this invention.

Generally, any vinyl aromatic monomer which is known to polymerize in free radical systems can be used. Such vinyl aromatic monomers typically contain from 8 to 20 carbon atoms. Usually, the vinyl aromatic monomer will contain from 8 to 14 carbon atoms. Some representative examples of vinyl aromatic monomers that can be utilized include styrene, 1-vinyl napthalene, 2-vinyl napthalene, 3-methyl styrene, 4-propyl styrene, t-butyl styrene, 4-cyclohexyl styrene, 4-dodecyl styrene, 2-ethyl-4-benzyl styrene, 4-(phenylbutyl) styrene, divinylbenzene and the like. Styrene is generally the most preferred vinyl aromatic monomer.

The alkyl acrylate monomers that can be used generally have the structural formula:



wherein R represents an alkyl group containing from 1 to 10 carbon atoms. The alkyl group in such alkyl acrylate monomers will preferably contain from 2 to 8 carbon atoms with alkyl groups which contain 4 carbon atoms being most preferred. Accordingly, ethyl acrylate, propyl acrylate, butyl acrylate, pentyl acrylate, hexyl acrylate and 2-ethyl hexyl acrylate are preferred alkyl acrylate monomers with butyl acrylate being the most preferred. The alkyl groups in such alkyl acrylate monomers can be straight-chained or branched. Thus, normal-propyl acrylate, isopropyl acrylate, normal butyl acrylate or tertiary-butyl acrylate can be employed. Normal-butyl acrylate is a particularly preferred monomer. The alkyl methacrylate monomers that can be used normally have alkyl groups which contain from 1 to about 20 carbon atoms. The alkyl methacrylate monomer will preferably have an alkyl group which contains from 2 to 12 carbon atoms. Some representative examples of alkyl methacrylate monomers which can be used include methyl methacrylate, butyl methacrylate, 2-ethylhexyl methacrylate, lauryl methacrylate and the like.

One particularly preferred polymer which can be made by the process of this invention is comprised of about 80 weight percent to about 95 weight percent vinyl aromatic monomers and from about 5 weight percent to about 20 weight percent conjugated diene monomers. It is particularly preferred for this polymer to contain from about 85 weight percent to about 92 weight percent vinyl aromatic monomers and from about 8 weight percent to about 15 weight percent conjugated diene monomers. It is also preferred for the vinyl aromatic monomer to be styrene and for the conjugated diene monomer to be 1,3-butadiene in these polymers.

Another highly preferred polymer which can be made by the process of this invention is comprised of about 70 weight percent to about 95 weight percent vinyl aromatic monomers and from about 5 weight percent to about 30 weight percent alkyl acrylate monomers. It is more preferred for such polymers to contain from about 85 weight percent to about 90 weight percent vinyl aromatic monomers and from about 10 weight percent to about 15 weight percent alkyl acrylate monomers. It is also preferable for the vinyl aromatic monomer to be styrene and for the alkyl acrylate monomer in these polymers to be butyl acrylate.

Such polymers will typically have glass transition temperatures which are within the range of about 45° C. to about 80° C. It is normally preferred for the polymer to have a glass transition temperature which is within the range of about 55° C. to about 70° C. with it being most preferred for the polymer to have a glass transition temperature which is

within the range of 60° C. to 65° C. As a general rule, higher levels of vinyl aromatic monomers result in higher glass transition temperatures. On the other hand, lower levels of vinyl aromatic monomers result in the polymer having lower glass transition temperatures. As a general rule, the glass transition temperature of the polymer should not be below about 40° C. because lower glass transition temperatures are indicative of polymers which are too soft for utilization in toner resin applications. The frangibility of toners is compromised if the glass transition temperature of the toner resin is above about 70° C.

Free radical emulsion polymerization techniques are utilized in conducting the process of this invention. Essentially any type of free radical generator can be used to initiate such free radical emulsion polymerizations. For example, free radical generating chemical compounds, ultra-violet light or radiation can be used. In order to ensure a satisfactory polymerization rate, uniformity and a controllable polymerization, free radical generating chemical agents are generally used. Some representative examples of free radical initiators which are commonly used include the various peroxygen compounds such as potassium persulfate, ammonium persulfate, benzoyl peroxide, hydrogen peroxide, di-t-butyl peroxide, dicumyl peroxide, 2,4-dichlorobenzoyl peroxide, decanoyl peroxide, lauryl peroxide, cumene hydroperoxide, p-menthane hydroperoxide, t-butyl hydroperoxide, acetyl acetone peroxide, dicetyl peroxydicarbonate, t-butyl peroxyacetate, t-butyl peroxyxymalic acid, t-butyl peroxybenzoate, acetyl cyclohexyl sulfonyl peroxide and the like; the various azo compounds such as 2-t-butylazo-2-cyanopropane, dimethyl azodiisobutyrate, azodiisobutyronitrile, 2-t-butylazo-1-cyanocyclohexane, 1-t-amylazo-1-cyanocyclohexane and the like; the various alkyl perketals, such as 2,2-bis-(t-butylperoxy)butane, ethyl 3,3-bis(t-butylperoxy)butyrate, 1,1-di-(t-butylperoxy) cyclohexane and the like. Persulfate initiators, such as potassium persulfate and ammonium persulfate are espe-

of such low molecular weight mercaptans results in odor problems. For instance, toners made with resins prepared utilizing such low molecular weight mercaptans can give off very unpleasant odors when the toner resin is ultimately used in a copier. Higher molecular weight mercaptans typically do not cause odor problems. However, they are not very effective at reducing the molecular weight of the polymer being prepared by free radical emulsion polymerization. It is typically advantageous for the chain transfer agent to be added incrementally throughout the polymerization.

The copolymerizations of this invention are carried out in the presence of a diacid cycloaliphatic emulsifier. These diacid cycloaliphatic soaps are typically cycloalkenes and cycloalkanes containing a carboxyl group and a fatty acid group bonded thereto, wherein the fatty acid group contains from 1 to about 25 carbon atoms. It is normally preferred for the diacid cycloaliphatic emulsifier to be of the structural formula:



wherein n is an integer from 1 to about 35, wherein m is an integer from 0 to 25 and wherein R<sup>1</sup>, R<sup>2</sup> and R<sup>3</sup> are selected from the group consisting of hydrogen atoms and alkyl groups containing from 1 to about 25 carbon atoms. Carboxy-4-hexyl-2-cyclohexene-1-octanoic acid which has the structural formula:



cially useful in such aqueous emulsion polymerizations. Hydrogen peroxide is also a highly preferred free radical initiator which can be used in the process of this invention.

Generally from about 0.1 phm (parts per hundred parts of monomer) to about 1.0 phm of initiator will be utilized to initiate the copolymerization. In most cases, about 0.2 to about 0.7 phm of a free radical initiator will be utilized. Preferably, about 0.3 phm to about 0.5 phm of a free radical initiator will be employed.

To reduce the molecular weight of the polymer, the emulsion polymerization can be conducted in the presence of one or more chain transfer agents. The chain transfer agent will typically be employed at a level which is within the range of 0.005 phm to about 6 phm. Alkyl mercaptans are particularly preferred for utilization as the chain transfer agent. Tertiary-dodecylmercaptan and normal-dodecylmercaptan are highly preferred with normal-dodecylmercaptan being the most highly preferred. Mercaptans having lower molecular weight alkyl groups cause dramatic reductions in molecular weight. However, the use

is a highly preferred diacid cycloaliphatic emulsifier.

The diacid cycloaliphatic emulsifier can also be a cyclohexane which is of the structural formula:



wherein n is an integer from 1 to about 35, wherein m is an integer from 0 to 25 and wherein R<sup>1</sup>, R<sup>2</sup> and R<sup>3</sup> are selected from the group consisting of hydrogen atoms and alkyl groups containing from 1 to about 25 carbon atoms.

The diacid cycloaliphatic emulsifier employed can also be in the form of a salt. Salts can be readily formed by reacting the diacid cycloaliphatic emulsifier with an appropriate base, such as sodium hydroxide, potassium hydroxide, ammonium hydroxide, monoethanol amine, diethanol amine or triethanol amine. As a general rule, sodium salts are preferred.

Generally, from about 0.5 phm to about 6 phm of the diacid cycloaliphatic emulsifier is utilized in preparing the aqueous polymerization medium. The use of less than about 0.5 phm of the diacid cycloaliphatic soap leads to latex instability. On the other hand, the utilization of more than about 6 phm of the diacid cycloaliphatic emulsifier causes isolation problems. In most cases, it will be preferred to utilize from 1 phm to 3 phm of the diacid cycloaliphatic soap. The precise amount of diacid cycloaliphatic emulsifier required in order to attain optimal results will, of course, vary with the monomers being polymerized. However, persons skilled in the art will be able to easily ascertain the specific amount of emulsifier required in order to attain optimal results. In some cases, it may be beneficial to add the diacid cycloaliphatic emulsifier incrementally as the polymerization proceeds.

The free radical emulsion polymerization will typically be conducted at a temperature which is within the range of about 100° F. (39° C.) to about 200° F. (93° C.). It is generally preferred for the polymerization to be carried out at a temperature which is within the range of 115° F. (46° C.) to about 175° F. (74° C.). To increase conversion levels, it is typically advantageous to increase the temperature as the polymerization proceeds. For instance, the polymerization temperature could be maintained at about 125° F. (52° C.) at the beginning of the polymerization and increased to a final temperature of about 175° F. (74° C.) at the end of the polymerization.

The polymerization time required in order to carry out such free radical emulsion polymerization generally ranges between about 3 hours and about 12 hours. In most cases, the polymerization reaction can be completed in about 4 to about 8 hours. The polymerization can be carried out as a batch process. However, it is generally advantageous to utilize a semi-continuous process wherein the monomers are charged over a period of about 2 to about 6 hours. It is typically most preferred to charge the monomers over a period of about 3 hours to about 5 hours.

After the polymerization has been completed, the toner resin can be recovered from the emulsion by coagulation. Divalent salts, such as calcium salts, magnesium salts, barium salts, zinc salts and the like can be used in the coagulation. Trivalent salts, such as aluminum salts, are generally better. The latex can be coagulated with alum (aluminum potassium sulfate) or an acid such as sulfuric acid, hydrochloric acid, nitric acid or acetic acid. It is highly preferred to coagulate the latex with sulfuric acid. It is not necessary to utilize salts or amines in such coagulation procedures. In fact, it is highly preferred to carry out the coagulation in the absence of salts or amines. This is because residual amounts of such compounds are detrimental to the ultimate properties of the toner resin. Hydrochloric acid can be used but is generally not preferred because it is too corrosive and can give off HCl gas. Nitric acid is also too corrosive and can give off nitrous oxide. The utilization of acetic acid can result in odor problems. For these reasons, sulfuric acid is highly preferred for utilization in carrying out the coagulation.

The cake of resin recovered by coagulation is then typically filtered and washed with water. It is then capable of

being dewatered by the process described in U.S. Pat. No. 2,615,206, known as syneresis. The teachings of U.S. Pat. No. 2,615,206 are incorporated herein by reference in their entirety. It is highly advantageous that the resins made by the process of this invention are capable of undergoing such a dewatering process. In this syneresis process, the cake of resin is simply heated to an elevated temperature which shrinks (contracts) the cake of resin thereby squeezing the water out of it. This syneresis process typically reduces the water content of the resin from about 70 percent to about 30 percent. The resin can then be further dried on an apron dryer.

Solid toners can be made with the toner resins of this invention utilizing standard procedures. Such toner resins will be comprised of the toner resin and at least one pigment, such as carbon black or iron oxide. In cases where carbon black is employed as the pigment, it will normally be present in the toner composition in an amount which is within the range of about 2 weight percent to about 10 weight percent. It is typically preferred for carbon black to be present in an amount which is within the range of about 5 weight percent to about 7 weight percent. In cases where iron oxide is employed as the pigment, it will normally be present in the toner composition in an amount which is within the range of about 10 weight percent to about 60 weight percent.

The toner composition can optionally contain a charge control agent and/or a wax. In cases where a charge control agent is used, it will normally be present in an amount which is within the range of about 0.5 weight percent to about 3 weight percent. In cases where a wax is included in the toner, it will typically be present in an amount which is within the range of about 1 weight percent to about 10 weight percent.

Liquid toner compositions can also be made utilizing the toner resins of this invention. Such liquid developer compositions are described in U.S. Pat. No. 5,572,274 and the teachings of U.S. Pat. No. 5,572,274 are incorporated herein by reference in their entirety. Such liquid toner compositions will normally be comprised of the toner resin, a liquid carrier and at least one pigment, such as carbon black or iron oxide. Appropriate colored pigments known in the art of liquid developer manufacture can also be used in making colored developer compositions. For instance, Sico Fast Yellow D1350 (BASF), Lithol Rubin D4576 (BASF), Lyonol Blue FG7351 (TOYO) and Lyonol Yellow 7G1310 (TOYO) can be utilized in amounts and combinations depending on the color and intensity desired. A list of additional colored pigments that are suitable for use is given in U.S. Pat. No. 4,794,651. The teachings of U.S. Pat. No. 4,794,651 are incorporated herein by reference in their entirety.

This invention is illustrated by the following examples which are merely for the purpose of illustration and are not to be regarded as limiting the scope of the invention or the manner in which it can be practiced. Unless specifically indicated otherwise, all parts and percentages are given by weight.

#### EXAMPLE 1

In this experiment, a toner resin was synthesized utilizing the emulsion copolymerization technique of this invention. In the procedure utilized, 17,490 grams of water, 1590 grams of a 20 percent aqueous solution of Diacid™ 1550 carboxy-4-hexyl-2-cyclohexene-1-octanoic acid emulsifier, 31.8 grams of sodium hydroxide, 31.8 grams of sodium sulfate, 1.3 grams of t-dodecyl mercaptan (a chain transfer agent) and 55.65 grams of ammonium persulfate were charged into a 10-gallon (37.85 liter) reactor. Then, the monomers were continuously charged into the reactor over a period of 4

hours at a rate of 8.9 pounds (4.0 kg) per hour. During this 4-hour period, 31.55 grams of styrene, 1590 grams of 1,3-butadiene and 206.7 g of t-dodecyl mercaptan were charged into the polymerization reactor as aqueous solutions. The monomer ratio of styrene to 1,3-butadiene was 89:11.

The polymerization temperature was maintained at about 130° F. (54° C.) with the solids content of the latex produced being monitored. After about 5 hours of polymerization time, when a solids content of about 40 percent was attained, the polymerization temperature was increased to about 165° F. (74° C.) and the polymerization was continued for an additional 3 hours. A final solids content of about 47 percent was attained after the full 8 hours of polymerization time.

The latex was then coagulated by pouring 5.5 pounds (2.5 kg) of it into 25 pounds (11 kg) of water which contained 25 grams of sulfuric acid at a temperature of 160° F. (71° C.). The resin was filtered out of the water, washed and dried at a temperature of 140° F. (60° C.) to a final moisture content of about 0.1 percent. The resin recovered in this experiment weighed 2.36 pounds (1 kg).

#### EXAMPLE 2

In this experiment, a toner was made utilizing the toner resin synthesized in Example 1. The toner was made by melt-mixing in an extruder 92 parts of the resin synthesized in Example 1 with 6 parts of Regal® 330 carbon black from Cabot Corporation and 2 parts of Arosurf™ TA-101 1-octadecanaminium, N,N-dimethyl-N-octadecyl-chloride charge control agent from Witco Corporation. The mixture was cooled, mechanically ground to about 1 mm granules and then pulverized on a jet mill to a medium volume particle size of about 10 microns to provide the toner.

Ricoh 610-type developer was obtained from Ricoh Corporation. Carrier beads were obtained by removing the Ricoh toner from the developer by either vacuuming through a 325 mesh sieve or washing with soap and water, rinsing several times with water, rinsing with isopropanol and drying the remaining beads.

The toner was combined with carrier beads at about 6 parts by weight of toner to 100 parts by weight of the carrier beads and was agitated until a positive triboelectric charge was produced on the toner particles. This mixture was then placed in a Ricoh FT 4215 copy machine which was modified to remove the fusing station. An unfused image was produced in this way. This image was passed through a fusing station from a Kodak 150 copier at a controlled rate of 0.5 feet (15.2 cm) per second and at a controlled temperature of 120° C.

Fusing quality was then measured by applying a strip of Scotch tape to a black image area, rolling a 1 kg weight over the tape three times and slowly removing the tape at a 180° angle. The optical density of the residual image was measured with a reflection densitometer. A residual density of 0.1 units is equivalent to blank paper (poor adhesion) and a density of about 1.3 is equivalent to solid black (excellent adhesion). By this method, the toner evaluated in this experiment had a residual optical density of 0.82 units.

For purposes of comparison, a toner resin having the same monomeric composition but made employing five parts of a conventional rosin acid soap was also synthesized. A toner was made utilizing this conventional toner resin. It had a residual optical density of only 0.28. Thus, the adhesion characteristics of toners can be greatly improved by utilizing diacid cycloaliphatic emulsifiers in the synthesis of the toner resin.

#### EXAMPLE 3

In this experiment, a styrene/butyl acrylate toner resin was synthesized utilizing the same general procedure as was employed in Example 1. However, the monomer charge consisted of 23 parts of butyl acrylate, 77 parts of styrene and 0.65 parts of divinyl benzene. In this experiment, the polymerization temperature was also increased to 172° F. (78° C.) and 1.0 parts of ammonium persulfate was employed to initiate the polymerization.

The toner resin synthesized was then compounded into a toner utilizing the procedure described in Example 2. The toner was then evaluated to determine adhesion characteristics utilizing the procedure described in Example 2 except for the fusion temperature being increased to 130° C. It was determined that the toner had a residual optical density of 1.09 units.

For purposes of comparison, a toner resin having the same monomeric composition but made employing two parts of sodium lauroyl sarcosinate soap was also synthesized. A toner was made utilizing this conventional toner resin. It had a residual optical density of only 0.30. Thus, this experiment again shows that the adhesion characteristics of toners can be greatly improved by utilizing diacid cycloaliphatic emulsifiers in the synthesis of the toner resin.

#### EXAMPLE 4

A black liquid developer can be prepared by mixing 10 parts by weight of the toner made by the procedure described in Example 1 and 5 parts by weight of Isopar L at low speed in a jacketed double planetary mixer connected to an oil heating unit for 1 hour with the heating unit being set at a temperature of 130° C.

A mixture of 2.5 parts by weight of carbon black and 5 parts by weight of Isopar L can then be added to the mix in the double planetary mixer and the resultant mixture can then be further mixed for about 1 hour at high speed. Then, 20 parts by weight of Isopar L preheated to 110° C. can be added to the mixer and mixed at high speed for about 1 additional hour. The heating unit can then be disconnected with mixing being continued until the temperature of the mixture drops to about 40° C.

The resultant mixture can then be transferred to an S-1 attritor device equipped with  $\frac{3}{16}$  inch carbon steel media, 45 diluted with Isopar L to a 16 percent solids ratio and ground without cooling until the temperature rises to about 60° C. Cooling, which can reduce the temperature to about 30° C. can then be commenced with grinding being continued for a total of about 24 hours. The mixture can then be removed 50 from the device and diluted with Isopar L to about 1.5 percent by weight solids concentration. The particles in the resultant toner concentration should have an average diameter of about 2.5 microns. A charge director can then be added to give the final liquid developer composition.

#### EXAMPLE 5

A liquid colored developer can be prepared by mixing 10 parts by weight of the toner resin made by the process described in Example 1 and 5 parts by weight of Isopar L at a low speed in a jacketed double planetary mixer connected to an oil heating unit for 1 hour with the heating unit being set to a temperature of 130° C.

Preheated Isopar L can then be added to reduce the solids concentration to preferably about 35 percent with mixing being continued at high speed for about 1 hour.

The mixture can then be transferred to an S-1 attritor device equipped with  $\frac{3}{16}$  inch carbon steel media with

## 11

pigment being added to the material in the attritor. The mixture can then be diluted with Isopar L to about a 12-16 solids ratio, depending on the viscosity of the material. Grinding can then be carried out without cooling until the temperature increases to about 60° C. Cooling, which will reduce the temperature to about 30° C., can then be continued for a total of about 24 hours. The mixture can then be removed from the device and diluted with Isopar L to a solids concentration of 1.5 weight percent. The particles in the resultant toner concentrate will have an average diameter of about 2.5 microns.

While certain representative embodiments and details have been shown for the purpose of illustrating the subject invention, it will be apparent to those skilled in this art that various changes and modifications can be made therein without departing from the scope of the subject invention.

What is claimed is:

1. A liquid toner which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers, (b) a residual amount of a diacid cycloaliphatic emulsifier, (c) a pigment and (d) a carrier liquid.
2. A liquid toner as specified in claim 1 wherein said liquid toner is further comprised of a charge control agent.
3. A liquid toner as specified in claim 1 wherein the toner resin does not contain residual levels of rosin acid soaps and wherein the toner resin does not contain residual levels of fatty acid soaps.
4. A liquid toner as specified in claim 3 wherein the polymer is prepared by a process which comprises (1) emulsion copolymerizing a vinyl aromatic monomer and a second monomer selected from the group consisting of conjugated diene monomers and an acrylate monomer selected from the group consisting of alkyl acrylate monomers and alkyl methacrylate monomers and (2) recovering the polymer from the aqueous emulsion.
5. A liquid toner as specified in claim 4 wherein from about 0.5 phm to about 6 phm of the diacid cycloaliphatic emulsifier is present during the copolymerization.
6. A liquid toner as specified in claim 1 wherein the vinyl aromatic monomer is styrene.
7. A liquid toner as specified in claim 6 wherein the second monomer is 1,3-butadiene.
8. A liquid toner as specified in claim 6 wherein the second monomer is selected from the group consisting of N-butyl acrylate and 2-ethylhexyl acrylate.
9. A liquid toner as specified in claim 7 wherein the repeat units in the polymer are derived from about 80 weight percent to about 95 weight percent styrene and from about 5 weight percent to about 20 weight percent 1,3-butadiene based upon total monomers.
10. A liquid toner as specified in claim 7 wherein the repeat units in the polymer are derived from about 85 weight percent to about 95 weight percent styrene and from about 8 weight percent to about 15 weight percent 1,3-butadiene based upon total monomers.
11. A liquid toner as specified in claim 8 wherein the repeat units in the polymer are derived from about 70 weight percent to about 95 weight percent styrene and from about 5 weight percent to about 30 weight percent of a member selected from the group consisting of N-butyl acrylate and 2-ethylhexyl acrylate.
12. A liquid toner as specified in claim 8 wherein the repeat units in the polymer are derived from about 85 weight percent to about 90 weight percent styrene and from about 10 weight percent to about 15 weight percent N-butyl acrylate based upon total monomers.
13. A liquid toner as specified in claim 4 wherein from about 1 phm to about 2 phm of the diacid cycloaliphatic emulsifier is present during the polymerization.
14. A liquid toner as specified in claim 4 wherein said copolymerization is initiated with a free radical initiator.
15. A liquid toner as specified in claim 14 wherein said free radical initiator is a persulfate initiator.
16. A liquid toner as specified in claim 14 wherein the free radical initiator is hydrogen peroxide.
17. A liquid toner as specified in claim 4 wherein said copolymerization is conducted at a temperature which is within the range of about 37° C. to about 93° C.
18. A liquid toner as specified in claim 17 wherein the polymer is recovered from the aqueous emulsion by coagulation with sulfuric acid.
19. A liquid toner as specified in claim 18 wherein said coagulation is carried out without utilizing salts or amines as coagulating agents.
20. A liquid toner as specified in claim 19 wherein water is removed from the polymer recovered by syneresis.
21. A toner resin which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers and (b) a residual amount of a diacid cycloaliphatic emulsifier, wherein said toner resin has a glass transition temperature which is within the range of about 45° C. to about 80° C.
22. A toner resin as specified in claim 21 wherein the toner resin does not contain residual levels of rosin acid soaps or fatty acid soaps.
23. A toner which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers, wherein said polymer has a glass transition temperature which is within the range of about 45° C. to about 80° C., (b) a residual amount of a diacid cycloaliphatic emulsifier and (c) a pigment.
24. A toner as specified in claim 23 which is further comprised of a charge control agent.
25. A toner as specified in claim 24 which is further comprised of a wax.
26. A toner resin as specified in claim 22 wherein the vinyl aromatic monomer is styrene.
27. A toner resin as specified in claim 26 wherein the second monomer is 1,3-butadiene.
28. A toner resin as specified in claim 26 wherein the second monomer is selected from the group consisting of N-butyl acrylate and 2-ethylhexyl acrylate.
29. A toner resin as specified in claim 27 wherein the repeat units are derived from about 80 weight percent to about 95 weight percent styrene and from about 5 weight percent to about 20 weight percent 1,3-butadiene, based upon total monomers.
30. A toner resin as specified in claim 27 wherein the repeat units are derived from about 85 weight percent to about 95 weight percent styrene and from about 8 weight percent to about 15 weight percent 1,3-butadiene, based upon total monomers.

## 12

percent to about 90 weight percent styrene and from about 10 weight percent to about 15 weight percent N-butyl acrylate based upon total monomers.

5 13. A liquid toner as specified in claim 4 wherein from about 1 phm to about 2 phm of the diacid cycloaliphatic emulsifier is present during the polymerization.

14. A liquid toner as specified in claim 4 wherein said copolymerization is initiated with a free radical initiator.

15. A liquid toner as specified in claim 14 wherein said 10 free radical initiator is a persulfate initiator.

16. A liquid toner as specified in claim 14 wherein the free radical initiator is hydrogen peroxide.

17. A liquid toner as specified in claim 4 wherein said copolymerization is conducted at a temperature which is 15 within the range of about 37° C. to about 93° C.

18. A liquid toner as specified in claim 17 wherein the polymer is recovered from the aqueous emulsion by coagulation with sulfuric acid.

19. A liquid toner as specified in claim 18 wherein said 20 coagulation is carried out without utilizing salts or amines as coagulating agents.

20. A liquid toner as specified in claim 19 wherein water is removed from the polymer recovered by syneresis.

21. A toner resin which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers and (b) a residual amount of a diacid cycloaliphatic emulsifier, wherein said toner resin has a glass transition temperature which is within the range of about 45° C. to about 80° C.

22. A toner resin as specified in claim 21 wherein the toner resin does not contain residual levels of rosin acid soaps or fatty acid soaps.

23. A toner which is comprised of (a) a polymer which is comprised of repeat units which are derived from a vinyl aromatic monomer and a second monomer selected from the group consisting of conjugated diene monomers and an acrylate monomer selected from the group consisting of alkyl acrylate monomers and alkyl methacrylate monomers, wherein said polymer has a glass transition temperature which is within the range of about 45° C. to about 80° C., (b) a residual amount of a diacid cycloaliphatic emulsifier and (c) a pigment.

24. A toner as specified in claim 23 which is further comprised of a charge control agent.

25. A toner as specified in claim 24 which is further comprised of a wax.

26. A toner resin as specified in claim 22 wherein the vinyl aromatic monomer is styrene.

27. A toner resin as specified in claim 26 wherein the second monomer is 1,3-butadiene.

28. A toner resin as specified in claim 26 wherein the second monomer is selected from the group consisting of N-butyl acrylate and 2-ethylhexyl acrylate.

29. A toner resin as specified in claim 27 wherein the repeat units are derived from about 80 weight percent to about 95 weight percent styrene and from about 5 weight percent to about 20 weight percent 1,3-butadiene, based upon total monomers.

30. A toner resin as specified in claim 27 wherein the repeat units are derived from about 85 weight percent to about 95 weight percent styrene and from about 8 weight percent to about 15 weight percent 1,3-butadiene, based upon total monomers.

**13**

**31.** A toner resin as specified in claim **28** wherein the repeat units are derived from about 70 weight percent to about 95 weight percent styrene and from about 5 weight percent to about 30 weight percent of a member selected from the group consisting of N-butyl acrylate and 2-ethylhexyl acrylate.

**32.** A toner resin as specified in claim **28** wherein the repeat units are derived from about 85 weight percent to about 90 weight percent styrene and from about 10 weight percent to about 15 weight percent N-butyl acrylate, based upon total monomers.

**33.** A toner as specified in claim **24** wherein the vinyl aromatic monomer is styrene.

**34.** A toner as specified in claim **33** wherein the second monomer is 1,3-butadiene.

**35.** A toner as specified in claim **33** wherein the second monomer is selected from the group consisting of N-butyl acrylate and 2-ethylhexyl acrylate.

**36.** A toner as specified in claim **34** wherein the repeat units are derived from about 80 weight percent to about 95 weight percent styrene and from about 5 weight percent to about 20 weight percent 1,3-butadiene, based upon total monomers.

**37.** A toner as specified in claim **34** wherein the repeat units are derived from about 85 weight percent to about 95

**14**

weight percent styrene and from about 8 weight percent to about 15 weight percent 1,3-butadiene, based upon total monomers.

**38.** A toner as specified in claim **35** wherein the repeat units are derived from about 70 weight percent to about 95 weight percent styrene and from about 5 weight percent to about 30 weight percent of a member selected from the group consisting of N-butyl acrylate and 2-ethylhexyl acrylate.

**39.** A toner as specified in claim **35** wherein the repeat units are derived from about 85 weight percent to about 90 weight percent styrene and from about 10 weight percent to about 15 weight percent N-butyl acrylate, based upon total monomers.

**40.** A toner as specified in claim **39** wherein the polymer has a glass transition temperature which is within the range of about 55° C. to about 70° C.

**41.** A toner as specified in claim **39** wherein the polymer has a glass transition temperature which is within the range of about 60° C. to about 65° C.

**42.** A toner resin as specified in claim **31** wherein the polymer has a glass transition temperature which is within the range of about 55° C. to about 70° C.

\* \* \* \* \*